

# UNITED STATES PATENT OFFICE.

CONRAD PAUL HUBERT CLAESSEN, OF BERLIN, GERMANY.

## GUNPOWDER.

No. 914,113.

Specification of Letters Patent. Patented March 2, 1909.

Application filed September 22, 1906. Serial No. 335,819.

*To all whom it may concern:*

Be it known that I, CONRAD PAUL HUBERT CLAESSEN, doctor of philosophy and chemist, subject of Prussia, residing at Dorotheenstrasse 45, Berlin, Germany, have invented new and useful Improvements in and Relating to the Manufacture of Gunpowder, of which the following is a specification.

This invention relates to smokeless powder for fire arms and ordnance. In many cases it has been proved advantageous in the case of powder of this kind to diminish the muzzle-flame, occurring when a shot is fired, or to entirely prevent the same. In order to attain this end, it is necessary to considerably lower the combustion-temperatures of the powder and to increase the ignition-temperature of the combustion gases produced when a shot is discharged. This purpose has hitherto been attained by an addition of indifferent or neutral bodies, such as vaseline, camphor or the like. Powders of very high combustion temperatures, such as nitrocellulose-nitroglycerin, powders, however, require for attaining this object the addition of such large quantities of such substances that the ballistic efficiency of the powder is so much decreased thereby as to render it valueless for practical purposes. One has already proposed, to obtain, by the addition to nitrocellulose-nitroglycerin powders of a mixture of indifferent or neutral bodies with small quantities of alkali bicarbonate, smokeless powder, which are practically free or nearly free of muzzle-flame and fulfil the ballistic requirements.

I have now found that smokeless nitrocellulose-nitroglycerin powder containing a

combination of small quantities of organic indifferent substances with small quantities (1-2%) of salts of the bibasic organic acids do not show the formation of muzzle-flames and have a sufficient ballistic efficiency and the stability of the said species of powders. As indifferent organic substances suitable for my purposes I have found oils, fats or resins. The skilled workman will select the substances suitable for this special purpose according to the price of the substances. As salts of the bibasic organic acids suitable for my purposes I have found the salts of tartaric, lactic, oxalic, malic, pyromucic, salicylic acid. The skilled workman will select the salts suitable for his special purpose according to the price of the substances.

As an example for a gunpowder according to my invention I quote the following.

|                   |       |                  |
|-------------------|-------|------------------|
| Nitrocellulose    | 69.88 | parts by weight. |
| Nitroglycerin     | 23.12 | " "              |
| Vaseline          | 5.00  | " "              |
| Potassium lactate | 2.00  | " "              |

Having thus described my invention what I claim as new and desire to secure by Letters Patent is—

An explosive consisting of an intimate mixture of nitrocellulose, nitroglycerin, vaseline and potassium lactate in substantially the proportions specified.

In testimony whereof I have signed my name to this specification in the presence of two subscribing witnesses.

CONRAD PAUL HUBERT CLAESSEN.

Witnesses:

HENRY HASPER,  
WOLDEMAR HAUPT.